

Jan. 12, 1943.

R. SOUKUP

2,307,863

SPINNING OF ARTIFICAL FILAMENTS

Filed Dec. 3, 1940

2 Sheets-Sheet 1

*Fig. 1*



*Roy Soukup*  
INVENTOR

BY *Louis Soukup*  
ATTORNEY

Jan. 12, 1943.

R. SOUKUP

2,307,863

SPINNING OF ARTIFICIAL FILAMENTS

Filed Dec. 3, 1940

2 Sheets-Sheet 2



Roy Soukup

INVENTOR

BY *Louis Adler*  
ATTORNEY

## UNITED STATES PATENT OFFICE

2,307,863

## SPINNING OF ARTIFICIAL FILAMENTS

Roy Soukup, Kenmore, N. Y., assignor to E. I. du Pont de Nemours & Company, Wilmington, Del., a corporation of Delaware

Application December 3, 1940, Serial No. 368,297

7 Claims. (Cl. 18—54)

This invention relates to a new and improved method for the spinning of viscose rayon yarn, i.e., regenerated cellulose yarn produced by the viscose process. More particularly, the present invention relates to a method of spinning viscose rayon yarn which comprises, coagulating the yarn in a first coagulating bath having an elevated temperature and continuing the coagulation in a second coagulating bath having a lower temperature than said first bath.

As a result of improvements and refinements in the method of spinning viscose rayon, the maximum permissible spinning speed has been gradually increased from less than 1,000 inches per minute to approximately 3,500 inches per minute. This increase in spinning speed has been made possible by numerous improvements in apparatus and process as well as improvements in raw materials and viscose and coagulating bath compositions. Such improvements have not only made possible an increase in the speed of spinning but they have also operated to yield a yarn of greatly improved physical characteristics. Both factors have contributed greatly to the increased production of viscose rayon yarn.

Despite the above-mentioned improvements, recent attempts to further increase the speed of spinning of viscose rayon yarn have had an adverse effect on the physical properties of the yarn. Heretofore, spinning speeds above about 3,500 inches per minute have been considered impractical. It has been found possible by greatly increasing the temperature of the entire coagulating bath to obtain satisfactory yarn at considerably increased spinning speeds. However, the bath temperature in such a case must be raised from the conventional spinning temperature of 40° to 50° C. to a temperature of the order of 80° to 90° C. The additional costs required to effect this change in temperature of spinning more than offset the advantages gained by the increase in spinning speed. Furthermore, rapid evaporation of water from the bath at the increased temperature causes the deposition of sulfate crystals from the bath solution upon machine parts, and also within the freshly spun yarn, thus leading to an excessive number of broken filaments within the yarn and increased maintenance cost of equipment.

The difficulty of operating the equipment in such a hot bath, and the fact that increased ventilation facilities are required when the entire bath is heated to such high temperatures, have also prevented the adoption of this method of spinning acceptable yarns at high speeds.

It is an object of the present invention to provide an improved method for the spinning of viscose rayon yarn.

It is a further object of this invention to provide an improved method for the spinning of viscose rayon yarn having a higher quality than may be produced by processes known heretofore.

It is another object of this invention to provide an economical and practical process for the spinning of viscose rayon yarn of suitable quality at greatly increased spinning speeds.

Other objects of the invention will appear hereinafter.

The objects of the present invention may be accomplished, in general, by extruding a solution of viscose from a spinneret into a coagulating bath maintained at an elevated temperature (at least 60° C.) and then passing the yarn for further coagulation and regeneration into a second bath maintained at a temperature much lower (at least 10° C. lower) than that of the first bath.

The yarn may be spun at high spinning speeds (at least 5,000 inches per minute) with the production of yarn of good quality.

The present invention will be more readily understood by reference to the following detailed description when taken in connection with the accompanying illustrations, in which:

30 Figure 1 is a graphic illustration showing the improvement in yarn quality to be obtained in accordance with the practice of the present invention.

Figure 2 is a perspective view of spinning apparatus suitable for use in accordance with the present invention.

Figure 3 is a perspective view of a modified form of apparatus suitable for use in accordance with the present invention.

40 Referring to the graphic illustrations shown in Figure 1 of the drawings, the several curves A, B, C and D illustrate the changes in the "quality factor" of viscose rayon yarn spun under varying conditions and at varying speeds and bath temperatures. The compositions of the viscose and the coagulating bath, or baths, were the same in all four curves.

Curve A illustrates the change in "quality factor" when viscose rayon yarn is spun at a spinning speed of 3,300 inches per minute into a coagulating bath having a temperature of 45° C. or greater and subsequently passing the yarn for further coagulation into a coagulating bath having a lower temperature.

55 Curve B illustrates the change in "quality

factor" of a yarn spun at a spinning speed of 3,400 inches per minute into a coagulating bath having a temperature of 35° C. or greater and in which the entire coagulation and regeneration of the yarn takes place in the one bath.

Curve C illustrates the change in "quality factor" of a yarn spun at a spinning speed of 5,300 inches per minute into a coagulating bath having a temperature of 35° C. or greater and in which the entire coagulation and regeneration of the yarn takes place in the one bath.

Curve D illustrates the change in "quality factor" when viscose rayon yarn is spun at a spinning speed of 5,300 inches per minute into a coagulating bath having a temperature of 27° C. or greater and subsequently passing the yarn for further coagulation into a coagulating bath having a lower temperature.

The term "quality factor" refers to the product of the dry tenacity and dry elongation of a particular yarn. This constitutes a reliable measure of the physical properties of the yarn. A high quality factor indicates a superior yarn due to improved physical properties. It is known that a change in spinning tension will alter the tenacity and the elongation of the yarn in opposite directions and if this change is not too great, the product of the two properties will remain approximately constant; hence, this product of tenacity and elongation is an expression of the total physical properties of the yarn.

The curves of Figure 1 of the drawings indicate that to duplicate, at a spinning speed of 5,300 inches per minute, the physical properties of a yarn obtained at 3,400 inches per minute in a bath at 45° C. (conventional spinning practice), the entire bath must be heated to 85° C. On the other hand, the curves show that a yarn of similar physical properties may be obtained at a speed of 5,300 inches per minute by spinning, in accordance with the present invention, in a system wherein that portion of the bath adjacent the spinneret is heated to a temperature of only about 60° to 70° C. while the remainder of the bath is kept at 45° C. When the bath near the spinneret is heated to still higher temperatures, the yarns spun in accordance with this invention are not only better than those spun at 3,400 inches per minute in a 45° C. bath, but are even better than those yarns spun at the lower speed when the entire bath is heated to any temperature.

An apparatus of the type shown in Figure 2 of the accompanying drawings may be satisfactorily used in the spinning of yarn according to the principles of this invention. In this apparatus a small tank 4 fitted with inlet and outlet tubes 5 and 6 is mounted within the coagulating bath trough 1. The coagulating bath trough 1 is fitted with inlet and outlet tubes 2 and 3. In one end of the tank 4, a small restricted opening 7 provides a passage, for the yarn spun in this tank, to the main bath trough. Hot bath is introduced continuously into this small tank through the tube 5 and discharged with the thread into the main trough or is led to drain through the outlet pipe 6. Additional bath of normal temperature is introduced into the main bath trough 1 through the inlet pipe 2. Bath is discharged from this trough through the pipe 3. The viscose solution is introduced into the small tank by means of the spinneret assembly 8. The freshly formed yarn 10 is led through a convergence guide 9 and through the opening 7 into the main bath trough where it is passed

around a guide 11 and then led from the trough to a collecting device 12.

Spinning apparatus for use in the practice of this invention differs from the standard viscose spinning machine only in that it possesses some means of maintaining at an elevated temperature that portion of the coagulating bath that immediately surrounds the spinneret. This means may satisfactorily comprise a small tank fitted within the main bath trough and containing the spinneret assembly as described above. However, it is not necessary that the freshly formed yarn pass directly from the hotter bath into the colder one. A system of rollers of the type shown in Figure 3 and which act to lift the yarn from the first bath and direct it into the second bath may be used. The second bath may, if desired, be provided with a multiple roller set-up whereby to obtain a long bath travel. As a further improvement, this small tank may be covered so as to prevent evaporation of the bath constituents.

A further modification contemplates the use of a hot bath into which only the face of the spinneret protrudes, the rest of the spinneret assembly being positioned in air or in a bath of normal temperature. Such a construction will act to prevent the gradual accumulation of gelled viscose within the spinneret assembly.

Other means may also be used. For instance, a spinning funnel of the type used in the spinning of yarn according to the cuprammonium process may be used in conjunction with a standard viscose spinning machine, the hot bath being contained within this funnel. Or, local heating may be supplied by mounting a heating device in the coagulating bath in close proximity to the spinneret.

With regard to other yarn properties, tests have shown that increasing the spinning speed and maintaining other conditions constant reduces the luster of the yarn slightly. However, the luster of the yarn spun with only that portion of the bath surrounding the spinneret heated, is equal to or better than the luster of yarn spun with the entire bath heated. The softness of the yarn is improved by the higher speed and still better results are obtained when the hot bath is confined to the region of the spinneret.

It is believed that the great improvements resulting from the practice of this invention are the result of a particularly favorable condition of coagulation at and near the face of the spinneret. They are not due simply to heating the viscose, for if the viscose inlet tube is surrounded with a steam coil, and the heated viscose is spun into a bath maintained at 45° C., distinctly adverse results are obtained. Neither are these improvements due only to the heating of the coagulated filaments for if the viscose is spun into an initial bath at 45° C. and the coagulated filaments are then passed into a hot bath, even though the initial 45° bath travel is less than 1/2 inch, the improvements are not obtained. Hence, it appears that some peculiar and hitherto unobserved effect occurring at the instant of coagulation of the viscose is responsible for the new results obtained by the practice of this invention.

Further evidence pointing toward the existence of such a peculiar type of coagulation in the practice of the present invention may be obtained from a study of the cuprammonium viscosities of yarns spun according to usual practice and according to the principles of the invention. The cupram-

monium viscosity of a yarn is a measure of the degree of degradation of the yarn, an increase in degradation being indicated by a decrease in cuprammonium viscosity. Tests reveal that yarns spun at 5,300 inches per minute and in accordance with the principles of this invention, possess a higher cuprammonium viscosity than do yarns spun from similar viscose into a 45° C. bath and at a normal draw-off speed of 3,200 to 3,400 inches per minute. This result is particularly evident when using viscose solutions of high salt index. Thus, the spinning of yarns by the process contemplated by this invention and at high spinning speeds, inhibits the degradation of the yarn that occurs when spinning at normal speeds and temperatures.

However, the cool (45° C.) portion of the bath does not serve only to cool the yarn passing through it. It also serves to permit the yarn to undergo further necessary chemical and physical reactions beyond the region of the heated spinneret zone. This is illustrated by the data of Tables I and I-A which show clearly that a certain minimum length of travel in a cool second bath containing the necessary chemical ingredients is necessary for the production of a satisfactory yarn. The data in these two tables are for yarn of 150-denier, 60-filament count, spun from cotton linters viscose containing 7% cellulose and 6% sodium hydroxide and ripened to a salt index of 5.2.

The data in Table I show the effect on yarn properties of passing the yarn from the heated bath directly into one or more cold baths of various compositions. In all cases, in this table, the yarn was spun at a speed of 6,810 inches per minute and first traveled a distance of 6½ inches through a bath heated to 95° C. and containing 11% sulfuric acid, 19% sodium sulfate, 4% glucose and 0.7% zinc sulfate before being passed through the cold baths and directed to a suitable collecting device.

In test No. 1, the yarn issuing from the hot bath was passed for a distance of 18½ inches through a second bath of the same composition as the hot bath, but maintained at a temperature of 45° C. This arrangement is in accordance with the preferred embodiment of the present invention.

In test No. 2, the yarn issuing from the hot bath was first passed for a distance of 28 inches through a second bath of the same composition as the hot bath but maintained at 45° C. The yarn was then further passed for a distance of 8¼ inches through a third bath containing small amounts (less than 2%) of sulfuric acid, sodium sulfate, glucose and zinc sulfate, and maintained at a temperature of 36° C.

In test No. 3, the yarn issuing from the hot bath was first passed for a distance of 10 inches through a second bath of the same composition as the hot bath, but maintained at 45° C. The yarn was then further passed for a distance of 8¼ inches through a third bath containing only small amounts (less than 3%) of sulfuric acid, sodium sulfate, glucose and zinc sulfate, and maintained at a temperature of 37° C.

In test No. 4, the yarn issuing from the hot bath was passed for a distance of 9½ inches through a bath containing only small amounts (less than 1%) of sulfuric acid, sodium sulfate, glucose and zinc sulfate, and maintained at a temperature of 33° C.

TABLE I

| 5  | Test No. | Spin tension | Break tension | Tenacity (dry) | Elongation (dry) | Quality factor | Grams per denier |       |          |
|----|----------|--------------|---------------|----------------|------------------|----------------|------------------|-------|----------|
|    |          |              |               |                |                  |                | Grams            | Grams | Per cent |
| 10 | 1        | 45.5         | 63.5          | 1.97           | 19.9             | 39.2           |                  |       |          |
|    | 2        | 60.3         | 80.0          | 2.23           | 17.0             | 37.9           |                  |       |          |
|    | 3        | 34.4         | 60.0          | 1.93           | 18.2             | 35.1           |                  |       |          |
|    | 4        | 12.5         | 20.0          | 1.55           | 18.9             | 29.3           |                  |       |          |

The data in Table I—A show the effect on yarn properties of changing the length of yarn travel in the cold bath. In all cases in this table, the yarn was spun at a speed of 5,400 inches per minute into a bath containing 11% sulfuric acid, 19% sodium sulfate, 4% glucose and 0.7% zinc sulfate and maintained at 85° C. The second or cold baths possessed the same composition as the hot bath in all cases, and were maintained at 45° C.

TABLE I—A

| 25 | Test No. | Hot bath travel | Cold bath travel | Spin tension | Break tension | Tenacity (dry) | Elongation (dry) | Quality factor | Grams per denier |       |          |
|----|----------|-----------------|------------------|--------------|---------------|----------------|------------------|----------------|------------------|-------|----------|
|    |          |                 |                  |              |               |                |                  |                | Grams            | Grams | Per cent |
| 30 | 5        | 6               | 1                | 16.2         | 28.3          | 1.52           | 22.5             | 34.4           |                  |       |          |
|    | 6        | 6               | 8                | 30.0         | 36.3          | 1.83           | 21.7             | 39.7           |                  |       |          |
|    | 7        | 6               | 14               | 31.0         | 76.0          | 1.92           | 22.1             | 42.3           |                  |       |          |
|    | 8        | 6               | 60               | 43.5         | 120.0         | 2.20           | 20.9             | 46.0           |                  |       |          |
|    | 9        | 5½              | 0                | 13.0         |               | 1.35           | 19.0             | 25.7           |                  |       |          |
|    | 10       | 5½              | 0                | 26.0         | 43.5          | 1.75           | 19.2             | 33.7           |                  |       |          |

35 A further striking fact that is brought out by the data of Tables I and I—A is the effect of the process contemplated by this invention on the breaking tension of the yarn. The breaking tension of present normal yarns spun at speeds of approximately 3,300 inches per minute in a bath maintained at 45° C. is approximately 35 to 55 grams. As shown in these tables, when the temperature of that portion of the bath surrounding the spinneret is heated to 95° C. and the remainder of the bath is maintained at 45° C. in accordance with the present invention, the breaking tension is raised to approximately 64 grams at 6810 inches per minute spinning speed and it is raised to 76 grams at 5,400 inches per minute spinning speed, and by increasing the yarn travel in the cool portion of the bath, as indicated in Table I—A, it is possible to increase the breaking tension of the yarn to 120 grams. This discovery, which further points to the existence of a peculiar type of coagulation in the case of this present process, is of the greatest practical importance. Not only does this improved breaking tension permit higher spinning tensions to be successfully employed in the spinning of yarns of higher tenacities, but, if only present normal spinning tensions are employed, it serves to promote improved spinning quality with a resultant decrease in the number of broken filaments, etc. because of the thus increased ratio of breaking tension to spinning tension.

70 The two tables above referred to disclose the improvement of the present invention when applied to the spinning of yarn at high spinning speeds. The present invention, however, has very distinct advantages in the spinning of yarn at speeds of the order of 3,000 inches per minute. Yarns spun at these speeds, in accordance with the present invention, are found to possess great-

ly improved physical properties. This is brought out most clearly by Table II below. The data contained in this table indicate the effect on the physical properties of yarns spun at a normal spinning speed of 3,300 inches per minute when the temperature of the bath surrounding the spinneret, and including the first six inches of bath travel is increased, while the temperature of the rest of the bath, or the second bath, is maintained at 45° C. In all cases, the total bath travel is 25 inches and the spinning tension is approximately 25 grams.

TABLE II

| Test No. | Bath temperature (spinneret zone) | Tenacity (dry)   | Elongation (dry) | Quality factor |
|----------|-----------------------------------|------------------|------------------|----------------|
| 1        | °C.                               | Grams per denier | Per cent         |                |
| 1        | 45                                | 1.76             | 20.9             | 36.8           |
| 2        | 66                                | 1.87             | 24.2             | 45.2           |
| 3        | 76                                | 1.86             | 25.2             | 46.9           |

By suitable manipulation of the spinning tension or bath travel, or both, the dry elongations of the yarn spun with the bath in the zone of the spinneret heated to temperatures of 66° C. and 76° C. may be reduced to a value of about 20.9% and the dry tenacities thereby increased to about 2.16 and 2.24 grams per denier, respectively. The essence of this process comprises spinning a viscous solution in to a hot bath with short travel, followed by a minimum length of travel in a cooler bath, and the process is not dependent upon spinning at a high rate of speed. Rather, one of the greatest advantages of the process lies in the fact that it makes possible the production of satisfactory yarn at high spinning speeds.

The following detailed examples are given to illustrate various methods for carrying out processes in accordance with the present invention. It is to be understood, of course, that these examples are not to be taken as limiting the invention.

## EXAMPLE I

Cotton linters viscose at a salt index of 4.0 and containing 7% cellulose and 6% sodium hydroxide is spun into a bath containing 11% sulfuric acid, 21% sodium sulfate, and 0.7% zinc sulfate, using a total bath travel of 25 to 30 inches at a spinning tension of 40 to 48 grams to give a yarn of 150 denier—60 filaments.

## Part A

The spinning speed is 3,400 inches per minute and the bath temperature 45° C., giving a dry tenacity of 2.17 grams per denier, a dry elongation of 17.4% and a quality factor of 37.8.

## Part B

The spinning speed is 5,300 inches per minute and the bath temperature 45° C., giving a dry tenacity of 1.84 grams per denier, a dry elongation of 16.8% and a quality factor of 30.9.

## Part C

The spinning speed is 5,300 inches per minute and the bath temperature 85° C., giving a dry tenacity of 1.98 grams per denier, a dry elongation of 18.3% and a quality factor of 36.2.

## Part D

The spinning speed is 5,300 inches per minute and the bath temperature for the first five inches of travel is 65° C. and thereafter is 45° C., giving a

dry tenacity of 2.13 grams per denier, a dry elongation of 18.9% and a quality factor of 40.3.

## Part E

5 The spinning speed is 5,300 inches, the bath temperature for the first five inches of travel is 85° C. and thereafter 45° C., giving a dry tenacity of 2.04 grams per denier, a dry elongation of 20.1% and a quality factor of 41.0.

## EXAMPLE II

Wood-pulp viscose at a salt index of 4.0 and containing 7% cellulose and 6% sodium hydroxide is spun in a bath containing 11% sulfuric acid, 19% sodium sulfate, 4% glucose, and 0.7% zinc sulfate, using a total bath travel of 25 to 26 inches to give yarn of 150 denier—60 filaments.

## Part A

10 The spinning speed is 3,300 inches per minute, the spinning tension is 30 grams, and the bath temperature is 45° C., giving a dry tenacity of 2.05 grams per denier, a dry elongation of 20.1% and a quality factor of 41.1.

## Part B

15 The spinning speed is 5,400 inches per minute, the spinning tension is 28 grams and the bath temperature is 45° C., giving a dry tenacity of 1.77 grams per denier, a dry elongation of 17.1% and a quality factor of 30.2.

## Part C

20 The spinning speed is 5,400 inches per minute, the spinning tension is 39 grams and the bath temperature is 82° C. for the first 5½ inches of travel and thereafter 45° C., giving a dry tenacity of 2.03 grams per denier, a dry elongation of 19.4% and a quality factor of 39.3.

## EXAMPLE III

25 The viscose, bath and spinning conditions in the respective parts are substantially the same as in Example II, except that the viscose is spun at a salt index of 6.0.

## Part A

30 The dry tenacity is 1.87 grams per denier, the dry elongation 20.2% and the quality factor 37.8.

## Part B

35 The dry tenacity is 1.60 grams per denier, the dry elongation 17.5% and the quality factor 28.0.

## Part C

40 The dry tenacity is 2.01 grams per denier, the dry elongation 21.0% and the quality factor 42.2.

## EXAMPLE IV

45 Wood-pulp viscose containing 7% cellulose and 4% sodium hydroxide and ripened to a salt index of 7.3 is spun into a bath containing 9.5% sulfuric acid, 22% sodium sulfate, 4% glucose and 0.7% zinc sulfate to give a yarn of 150 denier—60 filaments, using a total bath travel of approximately 25 inches.

## Part A

50 The spinning speed is 3,300 inches per minute, the spinning tension is 32 grams and the bath temperature is 45° C. The yarn possesses a dry tenacity of 1.63 grams per denier, a dry elongation of 17.4% and a quality factor of 28.4.

## Part B

55 The spinning speed is 5,400 inches per minute,

the spinning tension is 29 grams and the bath temperature is 45° C. The yarn possesses a dry tenacity of 1.52 grams per denier, a dry elongation of 14.8% and a quality factor of 22.5.

*Part C*

The spinning speed is 5,400 inches per minute, the spinning tension is 36 grams and the bath temperature is 83° C. for the first 5½ inches of travel and 45° C. for the remainder of the travel. The yarn possesses a dry tenacity of 1.94 grams per denier, a dry elongation of 21.0% and a quality factor of 40.7.

*EXAMPLE V*

Cotton linters viscose containing 7% cellulose and 6% sodium hydroxide and ripened to a salt index of 5.2 is spun to give a yarn of 150 denier—60 filaments at a draw-off speed of 8,850 inches per minute, using a total bath travel of 11 inches.

*Part A*

The spinning bath containing 11% sulfuric acid, 19% sodium sulfate, and 0.7% zinc sulfate is maintained at 47° C. It is impossible to spin yarn under these conditions.

*Part B*

The spinning bath possesses the same composition as Part A of Example V. The bath, for the first 5 inches of yarn travel, is maintained at 98° C., and for the remainder of travel is maintained at 46° C. The spinning tension is about 23 grams. The yarn possesses a dry tenacity of 1.46 grams per denier, a dry elongation of 21.5% and a quality factor of 31.4.

*Part C*

The spinning bath contains 12% sulfuric acid, 19% sodium sulfate and 0.7% zinc sulfate. The bath is maintained at 98° C. for the first 6 inches of yarn travel and at 46° C. for the remainder of the travel. The spinning tension is about 24 grams. The yarn possesses a dry tenacity of 1.51 grams per denier, a dry elongation of 22.4% and a quality factor of 33.8.

*EXAMPLE VI*

Cotton linters viscose containing 7% cellulose and 6% sodium hydroxide and ripened to a salt index of 5.2 is spun into a bath containing 12.5% sulfuric acid, 19% sodium sulfate, 4% glucose and 0.7% zinc sulfate at a spinning speed of 9,500 inches per minute to give a yarn of 150 denier—60 filaments, using a total bath travel of 13½ inches.

*Part A*

The entire spinning bath is maintained at 45° C. and the spinning tension is about 35 grams. The yarn possesses a dry tenacity of 0.74 gram per denier, a dry elongation of 7.5% and a quality factor of 5.6.

*Part B*

The spinning bath is maintained at 97° C. for the first 6½ inches of yarn travel and at 45° C. for the remainder of the travel. The spinning tension is about 21 grams. The yarn possesses a dry tenacity of 1.48 grams per denier, a dry elongation of 19.8% and a quality factor of 29.3.

The present invention is not limited to the use of a coagulating bath of any particular composition. Its advantages may be obtained with various types of baths, such as are well known in the art. Furthermore, it is not necessary that the two baths be of the same composition, or

even of the same general type. Preferably, however, the coagulating bath, or baths, employed in accordance with the present invention are of the type conventionally used in the commercial spinning of viscose rayon yarn and may contain, in addition to the usual 7% to 15% of sulfuric acid, glucose, ammonium sulfate, sodium sulfate, zinc, nickel or iron sulfate, etc. It is furthermore preferred, due to operating convenience, that the two baths be of the same composition thereby permitting the small quantity of hot bath immediately surrounding the spinneret to flow into the larger bath trough to heat the same.

As indicated by the examples contained in this specification, the process contemplated by this invention is not limited to the use of a viscose solution of any specified composition or degree of ripeness. In fact, one of the advantages of the process lies in the fact that it enables yarns of satisfactory and even improved properties to be spun from viscose solutions that have been ripened less than a normal time. For example, yarn spun from a wood-pulp viscose of salt index 3.0 at 5,400 inches per minute spinning speed, with a 5-inch travel at the spinneret in a bath heated to 82° C. and with the main bath at 46° C., possesses a dry tenacity of 2.06 grams per denier and a dry elongation of 16.0% for a quality factor of 33.0. Yarn spun under similar conditions but using a viscose solution with a salt index of 4.1 possesses a dry tenacity of 2.09 grams per denier and a dry elongation of 17.6% or a quality factor of 36.8, while yarn spun from a viscose solution with a salt index of 7.1 possesses a quality factor of 43.0.

The results obtained in this manner are very striking and are of tremendous importance. It has been suggested in the past that it should be possible to substantially increase the quality factor of a viscose rayon yarn by the use of a viscose solution of high salt index. The chief difficulty in achieving such an increase in the past has been the inability to obtain a spinning bath which will effect a sufficiently rapid and uniform "setting-up" of the gel structure of the yarn early in the spinning process. The above results indicate clearly that the use of a hot bath in the region of the spinneret provides, for the first time, such a desired condition. This process not only permits viscose solutions of high salt index to be used in the spinning of yarns of improved properties, but it has been found possible when operating in accordance with this invention to reduce the tendency toward bad spinning and plugged spinnerets by increasing the salt index of the viscose solution.

Naturally, when viscose solutions of different compositions or degrees of ripeness are employed, it may be desirable to alter to some extent the various factors involved in the spinning operation, such as spinning tension, bath travel, etc. For instance, it is found, when using a viscose solution possessing a higher than normal salt index, that it is desirable to increase somewhat the length of travel of the yarn in the heated portion of the bath. The invention contemplates that such changes in these factors as are found necessary to obtain the optimum spinning conditions will be made.

The optimum length of travel of the yarn in the hot bath depends on various factors, such as the composition of the viscose solution and coagulating bath, the type of yarn being spun, the spinning speed, the hot bath temperature, and the desired relationship between tenacity and

elongation. For the conditions of Example I, Part E, the tenacity is greatest with a short hot bath travel of 1 to 4 inches and decreases rather rapidly with longer travel until at 15 inches hot bath travel, it is only 80% of its maximum value. The elongation has a maximum value at 7 to 12 inches hot bath travel, but falls only slowly at longer travels. The maximum quality factor is obtained at about 5 inches travel. These effects provide a certain flexibility in the process. If a 10 yarn of maximum tenacity and somewhat reduced elongation is desired, a travel of 2 or 3 inches in the heated bath will be preferred. For 15 yarn of higher elongation and reduced tenacity, a travel of about 10 inches is better. It is also possible to obtain yarn of the maximum quality factor by spinning with a bath travel of 5 inches and adjusting the elongation and tenacity by altering the spinning tension. In general, the travel of the yarn in the hot bath is preferably 20 relatively short and will vary from 1 to 10 inches.

The conditions stated above concerning the length of travel in the heated bath hold regardless of the length of travel of the yarn in the second bath, which length may be varied greatly above a certain minimum value indicated in 25 Table I without seriously affecting the properties of the yarn. In any case, the length of travel in the second bath will be dependent upon such factors as temperature of the bath, spinning tension, type of yarn spun, etc. In general, the travel of the yarn in the second, or cooler, bath is considerably greater than the length of travel 30 in the hot bath. Depending upon the physical characteristics which it is desired to impart to the yarn, the yarn will be passed through the second bath a distance of between 12 to 50 or more 35 inches.

To obtain the advantages of this invention, the temperature of the first bath must be raised to at least 60° C. Even greater advantages accrue if the temperature of this bath is raised to a temperature of 85° C. or 100° C. or even higher. These higher temperatures will be of the greatest importance when spinning at speeds of the order of 7,000 inches per minute or more, and particularly, when spinning at speeds of the order of 10,000 inches per minute or more. In connection with these very high speeds, it may be desirable to add various substances, such as glucose or 40 glycerin, to the bath, so that it may be heated to a sufficiently high temperature.

In this connection, it might be noted that the use of the hot spinning bath reduces the liquid drag on the yarn passing through the bath and on the guide rollers rotating in the bath. The spinning tension specified in Parts A and B, respectively, of Example VI illustrate this effect, which is due to the lowered viscosity of the heated bath. Thus a useful means is provided for at least partially controlling the substantial increase in spinning tension which is encountered with the increased spinning speeds with which this invention is concerned. Because a high spinning tension has an adverse effect on spinning performance and physical properties of the yarn, the reduction in liquid drag made possible by the use of a heated bath is of the utmost importance in the spinning of a satisfactory yarn at high speeds.

In accordance with the principles of this invention, the temperature of the second bath must be lower than that of the first bath and should preferably be of the order of 45° C. or even lower. Temperatures much above 45° C. in the second

5 bath will lead to the disadvantages obtained when the entire bath is heated. The optimum temperature of the second bath will depend upon the exact spinning conditions encountered, including the temperature of the first bath and the relative length of travel of the yarn in the two baths. However, any reduction in temperature between the first and second baths will be better than the use of a single hot bath. The temperature of this second bath should be maintained at least 10° C. below that of the first bath and should preferably be of the order of 45° C. or even lower.

15 The examples contained in this specification disclose the spinning of viscose rayon yarn at speeds up to 9,500 inches per minute. However, the advantages of the invention may also be realized at higher speed, such as 12,000 inches per minute or even higher as, for example, upwards of 15,000 inches per minute.

20 This invention is not limited by the extent or manner of applying tension during the spinning operation. When spinning yarn in the two-temperature bath system of this invention and maintaining the spinning tension constant, it is found that an increase in the temperature of the first bath causes a small increase in tenacity and a considerably greater increase in elongation. Hence, the invention contemplates the increase of the spinning tension by an amount sufficient to increase the tenacity of the yarn in a manner corresponding to the increase in elongation. However, the invention also contemplates the use of other means than an increase in spinning tension to gain this increase in yarn tenacity. For example, the invention contemplates subjecting the finished yarn to a stretching operation in a third bath maintained at an elevated temperature in accordance with the procedure outlined in the copending application U. S. Serial No. 278,403 to Karns, filed June 10, 1939.

25 The chief advantage of this invention lies in its ability to produce yarn of better physical properties than can be obtained either with the entire bath heated to the preferred temperature or with the entire bath maintained at the temperatures now employed in commercial spinning processes. The invention is most useful when spinning at high speeds because improvements in physical properties are greatly needed under these conditions. The essential feature of the invention consists in maintaining the spinning bath in the region of the spinneret face and for 30 a distance of from 1 to 10 inches beyond at a temperature above 60° C. while maintaining the main body of the bath at a lower temperature.

35 When contrasted with that process in which the entire bath is maintained at an elevated temperature, the process contemplated by this invention is found to possess the following advantages:

1. For the same maximum temperature this invention produces a yarn of superior physical properties.
2. To obtain equivalent properties, the required maximum temperature is substantially lower.
3. Since the high temperature bath is confined to a small volume through which a rapid flow may be economically provided, an adequate control of temperature may be obtained.
4. This invention requires that only a small portion of the entire coagulating bath be heated to an elevated temperature. The trough containing this small section may be easily thermally insulated and the hot bath carried away by the

spinning filaments may be utilized to heat the main bath to the desired temperature. Heat losses are consequently not important.

5. The surface of the hot bath is relatively small and may be covered. In this manner, evaporation losses are reduced to a minimum.

6. The major portion of the bath is maintained at lower temperatures and thus the yarn is cooled before it leaves the bath. Hence, the tendency toward crystal formation within the yarn is no greater than at the present time. In fact, inasmuch as this invention contemplates the use of a main bath at a temperature below 45° C., this tendency toward crystal formation will be greatly reduced over the present standard. This is a very important advantage inasmuch as it offers a great decrease in the number of cut and broken filaments.

7. Except for actually starting the flow of filaments from the spinneret face, all the manipulations of the operators are carried out at normal temperatures. The gross machine parts, the guides, bobbins, etc., and the unavoidable spray and drip from the moving parts are not hot. This is a tremendous advantage from the viewpoint of practical, economical operation and maintenance.

8. The process contemplated by the present invention is operative with any bath that can be used in present normal practice. The process requires no difference in composition between the two baths although such a difference may prove to be desirable for other reasons and is contemplated by the invention.

The process provides a means of adjusting the tenacity and elongation of the product by simply changing the length of travel of the yarn in the hot bath.

The process provides a means whereby undesirably large increases in spinning tension may be avoided as the spinning speed is increased.

The process also provides a means of increasing the breaking tension of the yarn during the spinning operation. This increase is desirable because it not only permits a higher spinning tension to be employed whereby the yarn possesses a greater tenacity, but it also serves to improve the spinning quality when only normal spinning tension is employed, thus reducing the number of broken filaments in the spun yarn.

The process provides a means of producing an improved product by the use of a viscose solution ripened to a degree less than normal.

Cuprammonium viscosity measurements show that yarn produced by this process is degraded to a smaller extent than is yarn produced according to known processes.

Although this discussion of the invention has been limited to the spinning of yarns from a viscose solution, it is obvious that the invention should not be so limited. Its principles can be used successfully in the manufacture of films, tubings and other structures of regenerated cellulose from viscose solutions. Such articles, prepared in accordance with the principles of this invention, will be found highly suitable for use in the art.

Since it is obvious that many changes and modifications can be made in the details above described without departing from the nature and spirit of the invention, it is to be understood that the present invention is not to be limited to the said details except as set forth in the appended claims.

I claim:

1. A process of spinning viscose rayon yarn which comprises extruding the viscose through a spinneret into an acid coagulating bath containing 7% to 15% sulfuric acid and having a temperature of at least 60° C., and passing the resulting yarn, at a speed of at least 5,000 inches per minute, into a second coagulating bath having a lower temperature than the first bath.
- 10 2. A process of spinning viscose rayon yarn which comprises extruding the viscose through a spinneret into an acid coagulating bath containing 7% to 15% sulfuric acid and having a temperature of at least 60° C., and passing the resulting yarn, at a speed of at least 5,000 inches per minute, into a second coagulating bath having a temperature of at least 10° C. lower than the first bath.
- 15 3. A process of spinning viscose rayon yarn which comprises extruding the viscose through a spinneret into an acid coagulating bath containing 7% to 15% sulfuric acid and having a temperature of at least 60° C., and passing the resulting yarn, at a speed of at least 5,000 inches per minute, into a second coagulating bath having a temperature of the order of 45° C.
- 20 4. A process of spinning viscose rayon yarn which comprises extruding the viscose through a spinneret into an acid coagulating bath containing 7% to 15% sulfuric acid and having a temperature of at least 60° C., moving the resulting yarn through said bath for a distance between 1 and 10 inches, and passing the resulting yarn, at a speed of at least 5,000 inches per minute, into a second coagulating bath having a lower temperature than the first bath.
- 25 5. A process of spinning viscose rayon yarn which comprises extruding the viscose through a spinneret into an acid coagulating bath containing 7% to 15% sulfuric acid and having a temperature of at least 60° C., moving the resulting yarn through said bath for a distance between 1 and 10 inches, and passing the resulting yarn, at a speed of at least 5,000 inches per minute, into a second coagulating bath having a temperature of at least 10° C. lower than the first bath.
- 30 6. A process of spinning viscose rayon yarn as defined in claim 1 in which the composition of the second coagulating bath is substantially the same as the first coagulating bath.
- 35 7. A process of spinning viscose rayon yarn as defined in claim 2 in which the composition of the second coagulating bath is substantially the same as the first coagulating bath.

ROY SOUKUP.